

W. M. PAGE.  
PROCESS OF MAKING CLAD TUBULAR ARTICLES.  
APPLICATION FILED APR. 20, 1910.  
**1,125,159.**

Patented Jan. 19, 1915.



Inventor

William M. Page

Witnesses  
H. G. Robielle  
H. Schoenthal

By K. P. McElroy  
Attorney

# UNITED STATES PATENT OFFICE.

WILLIAM MARSHALL PAGE, OF PHILADELPHIA, PENNSYLVANIA.

## PROCESS OF MAKING CLAD TUBULAR ARTICLES.

1,125,159.

Specification of Letters Patent.

Patented Jan. 19, 1915.

Application filed April 20, 1910. Serial No. 556,602.

*To all whom it may concern:*

Be it known that I, WILLIAM MARSHALL PAGE, a citizen of the United States, residing at Philadelphia, in the county of Philadelphia and State of Pennsylvania, have invented certain new and useful Improvements in Processes of Making Clad Tubular Articles, of which the following is a specification.

10 This invention relates to processes of making clad tubular articles; and it comprises a method wherein a hollow or tubular body of ferrous or like metal is heated from one side to a suitable temperature and while 15 so heated is united to a body of copper or like metal; all as more fully hereinafter set forth and as claimed.

For heat-exchanging elements, such as boiler tubes, and for many other purposes, 20 the value of copper-clad steel is evident. In a boiler tube, for example, the strength of steel and the heat-conductive and corrosion-resisting properties of copper are desirable. Steel corrodes and oxidizes easily and is 25 relatively a poor conductor for heat. In a boiler tube there is little lateral conduction of heat though this would obviously be advantageous as equalizing the temperatures and diminishing the tendency of scale to 30 bake on. Most of the heat from impinging flame gases is localized, little spreading laterally from each point of impingement, so that part of the tube is not actively functioning while the residue is pushed to 35 duty. As the amount of heat transmitted through a metal wall in a time unit is a compound function of the relative conductivity of the metal and the difference in temperature between the two sides, or "heat

40 head," this means that the high temperature gases first impinging do not transmit as much heat in the time afforded as they should while being cooled somewhat on subsequent exposure to the rest of the boiler 45 tube, heat transfer becomes slowed up. And at the spot of localized high temperature where heat transfer is active, scale is apt to bake on. With a copper tube on the other hand, there is an active lateral trans-

50 mission of heat from any spot of localized high temperature so that with copper there is not only a better and more active trans-

mission of heat at the point where the furnace gases strike the boiler tube but also the zone of active heat transmission is broadened out laterally. More of the tube is 55 actively functioning. Copper is also highly resistant to corrosion, either by boiler waters or by furnace gases. But copper is a comparatively weak, soft metal. 60

It is not desirable to make a mere assemblage of concentric tubes of the two metals for boilers, partly because their expansion and contraction are so widely different and partly because the line of non-union or seam 65 between such tubes would tend to prevent efficient transmission of heat. For quick transmission of heat, the two metals must be in metallic contact. In such an assemblage, furthermore, both metals must be 70 present in sufficient thickness to give each layer of metal substantial strength of its own. Ordinarily copper-plating by electrolytic methods does not give an efficient article for this purpose, electro-deposited 75 coatings being invariably porous, crystalline, and of little real adherence to their base, from which they tend to part on heating. Copper and steel forming an excellent galvanic couple, the presence of the 80 porous copper tends to aid corrosion. For purposes like the present, the two metals must be in an absolute metallic union which is, or is equivalent to, a weld union so that 85 they may not shrink apart and that they may transmit heat efficiently while the copper must be wholly impervious so that corrosive agents cannot reach the steel.

Joined copper and steel united by a union 90 of this character have long been desired in the art; but until recently have not been produced. Copper and steel are so unlike in chemical and physical nature that they cannot be united by simple heat and pressure in the way in which iron can be united 95 to iron or even copper to copper. To produce a firm union between metals they must be in a contact which is, or is equivalent to, a molecular contact and to secure this one or both the metals must be in a molten or at 100 least fluent condition so that a liquid contact, or "wetting contact," can be secured. And such an intimate contact is not easily to secure between steel and copper.

In the elder art, most of the attempts to weld-unite copper and steel failed from a lack of recognition of this fact. Hot-rolling the two metals together was often tried but 5 gave at most a mere fitting together or adhesion in lieu of a cohesion, never producing inseparably united metals, and the many attempts at casting the two metals together fared no better. In casting copper against 10 steel under ordinary casting conditions for example, it is probable that no real metallic contact of the nature of a wetting contact ever resulted; partly, probably, because copper has little chemical or physical affinity 15 for steel and does not readily "wet" it. If the steel body were hot it was usually oxidized on the surface with the oxid forming a physical spacing layer which prevented the liquid copper coming into actual contact 20 with the steel while as the cast liquid copper solidified in the mold the gases evolved in solidifying went to the center; to the line between the hot steel core and the still molten parts of the copper. If the steel were 25 clean and cold, the copper cast against its surface solidified there before time was afforded for any actual contact or even for displacement of "absorbed" gases. Of late however it has been possible to attain true 30 weld unions as by the methods described in Patent 853,716 where the copper is contacted with the steel in a superheated or supermolten condition; under which circumstances it readily wets and unites with it, 35 forming unions which are, or are in the nature of, true weld unions. After cooling, good welds so effected are inseparable save by heat sufficient to melt off the copper, a cleaving tool, such as cold chisel, or heating 40 and quenching, failing to discover any line or seam of non-union and the joined metals may be rolled, drawn, swaged, spun and otherwise worked like a body of a single metal. It is however difficult and expensive 45 to roll or manufacture tubing and tubular articles directly from non-tubular shapes of clad metals; and there is a difficulty peculiar to clad metal in forming such articles from tubularly bent sheets in that a double union 50 must be formed at the seam to attain full strength. The operation is not so simple as forming hollow articles from steel or iron sheets or bars. In the present invention however I have devised a simple, cheap and 55 ready method of directly forming steel or iron tubing and hollow articles clad with a coating of integrally and metallically united copper, or metal comprising copper, and with a union therebetween which is, or is 60 equivalent to, a weld union. For this purpose I first prepare a steel or iron tube or hollow article of nearly the final dimensions required and then expose it to heat from one side while another side is in contact with a

body of copper until the proper thermal and 65 other conditions requisite for union between steel and copper are produced on the side of the steel in contact with said copper. Or, in other words, I heat through the ferrous metal wall until proper heat and other 70 conditions occur on the other side to produce the desired union between the ferrous metal and a proximate layer of molten copper.

The heating may be by any convenient 75 method or apparatus using fire or flame heat, electrical heating or even the heat of solid fuel. An oil or gas flame is, however, well adapted for use for the present purposes, such flame being, for instance, directed 80 through or into the tubular or hollow body, or around it when the interior is to be clad. The article may be either interiorly or exteriorly clad with copper. The copper may be brought into contact with the ferrous 85 metal article to be clad or coated in any convenient manner, as by casting copper, or by placing a solid copper body of appropriate shape, thereagainst. Or, in the case of an exterior coating, copper wire may be wound 90 around the article; or a suitable surrounding mold casing may be filled with chips, or other forms of finely divided copper. The article may receive a preliminary copper coating electrically. The coating metal in 95 lieu of being pure copper may be any cupriferous alloy, such as brass. Brass while readily attached to steel by the methods of Patent 853,716, is not readily rolled and otherwise worked at steel working temperatures, but as in the present invention no extensive subsequent working is necessary, the present method gives a convenient method of 100 making brass clad tubular articles. Aluminum bronze and other bronzes may be 105 used. A good coating material for many purposes is what may be termed an iron bronze; an alloy of copper and iron. While copper and iron stand far apart in the electrical scale so that copper promotes the 110 corrosion of steel yet various of the iron bronzes are electrically neutral to iron and steel, being neither substantially positive or negative thereto, while they are, like copper, very 115 resistant to corrosion. If desired, a layer of linking low melting metal may be used to facilitate the union, the steel article being, for example, first galvanized, tinned or sherardized.

Where the coating is to be interior, a 120 blocking out mold of appropriate form may be employed to constitute with the interior of the article an annular mold. The steel or iron article to be clad or coated may first be sandblasted, pickled and cleansed, or it 125 may be left covered with furnace scale; which consists mainly of ferrosoferric oxid and may have a useful function in the union,

as hereinafter explained. An inert or reducing atmosphere, such as producer gas or water gas, may be maintained around the side to be coated or clad during the operation; or this side may be bathed in or coated with suitable flux, such as an alkaline body like waterglass or borax or one of the halogen compounds, such as sodium chlorid, fluorspar, cryolite, calcium chlorid, etc.

Under the described conditions, the copper or other metal in contact with the steel may be melted and raised to any suitable temperature, such as the supermolten temperature, or it may, of course, be melted prior to bringing it in contact with the steel and then further heated, or its heat maintained, during the operation. Under the described conditions since the maximum temperature of the copper will prevail along the line of intended union, and any desired time for solidification may be given, the described difficulties incident to the ordinary casting operation do not occur. The copper layers most remote from the steel may be caused to solidify first. Where high conductivity, either for heat or electricity, is desired, it is a useful expedient at times to keep these outer layers cooled below the melting point as in such event any contamination of the layers beyond those next the steel with dissolved iron cannot occur. The presence of iron in copper reduces its heat conductivity out of all proportion to the amount of such iron. The steel may of course be preliminary film coated with copper or copper iron alloy by the methods described in Patent 853,716.

A useful preliminary to the operation is to produce more or less pure iron on the surface of the steel. Iron unites with copper very much more readily than does steel, and at lower temperatures, the presence of the carbon in the steel materially reducing the tendency toward union. In this preliminary treatment, the steel object may, for instance, be first oxidized and then re-reduced, as by exposing it in a heated condition to an atmosphere of producer gas. In the oxidation, the superficial carbon burns out more or less thoroughly and the iron reduced from the oxid is substantially pure. A better way, however, is to first treat the steel by exposure to superheated streaming steam which causes the formation of a thin, closely cohering coating of a ferrosoferric or magnetic oxid on its surface. This coating coheres much better to steel than do ordinary oxid coats and is in molecular contact with the underlying metal. By now heating, the underlying superficial carbon of the steel reduces this oxid, forming pure iron both from the oxid and also from the underlying layers. With this pure iron, copper readily unites. The heat of molten copper is suffi-

cient to perform the oxid-reducing reaction and the point where the union of copper and steel is completed may be told by the cessation of bubbles of liberated oxides of carbon. With a clean steel billet and with copper containing, as it usually does, both dissolved oxid and oxygen, instead of first oxidizing the steel, the oxygen in the copper may be employed to burn out the superficial carbon of the steel and produce the desired pure iron.

A useful specific way of performing the present invention, assuming that an exteriorly clad tube is required, is to sandblast and pickle a steel tube, which may be of any steel desired and made in any desired manner as by lap welding, Mannesmann drawing, etc., and then expose this tube to superheated streaming steam, as by placing it in a heated casing into which steam is introduced. It soon heats up and becomes covered with the described coating of oxid. This tube may now be placed in a sand mold, copper cast around it, and the heat of a suitable flame directed through it until its exterior layer is at a suitable temperature and the desired union with the copper is attained. Or the tube may be cleaned, sandblasted and pickled to obtain a true metallic surface and then copper containing oxygen cast or flowed around it in a suitable mold while interiorly heating until union is effected. Or the cleaned tube may be simply interiorly heated in contact with pure copper until such copper is not only melted but becomes supermolten. After the union is effected, the clad tube may be removed and given a final pass or two to reduce it somewhat in gage and to compact the coating. It may, for example, be cold drawn. This working has the useful effect of producing an advantageous physical change in the coating metal which being compacted between the working tool on the one side and the relatively stiff hard metal on the other while held against lateral yielding by the existence of a basal weld union, assumes throughout its mass a peculiar texture comparable with the surface texture of hard drawn wire. This much improves it for most purposes requiring strength and a good surface.

In an article of the present nature, the two metals are in absolute metallic union with a union which is, or is equivalent to, a weld union, resisting discovery by cleaving tools, such as a cold chisel, or by the effect of heating and quenching. The two metals do not part by the influence of temperatures short of the melting point of the coating metal. And for heat transferring purposes, as in boiler tubes and the like, the presence of the layer of copper whether interior or exterior much improves the effi-

ciency by providing for a lateral spreading and equalizing of heat in a way impossible with an all-steel article.

Where it is desirable, as it often is, that the metal of the coating shall not be contaminated to any extent by dissolved iron, the coating layer may be cold on the side removed from the iron or steel. For example, in producing a tube clad with an outer copper layer, the copper may be cast into contact with the interiorly heated tube in a mold having cooling means in the wall. By properly controlling the cooling, the outer layers of the copper coating may be solidified and kept solidified while the layers next the iron or steel are left liquid and form the union with the ferrous metal. Or a sleeve of copper surrounding the iron or steel may be melted in the layers in contact with such iron or steel while the exterior layers of copper or those next the mold walls may be kept solid. Operating in this manner there is no danger of a diffusion of dissolved iron outward into the main body of the coating.

In the accompanying illustration I have shown, more or less diagrammatically, in central vertical section, one embodiment of the described invention.

30 In this showing element 1 is an annular mold of any suitable material strengthened by steel bands 2. At its bottom, it is provided with a recess wherein seats an annular steel body 4. In the chamber between the 35 annular steel body and the mold is a body of copper 5. Covering this body may be a cover 6. Flame producing means 7 are adapted to direct a brush flame of oil, gas or the like within the annular steel body. 40 Above the flame chamber is hood 8 for removal of gas.

The use of the apparatus shown is obvious from the foregoing. Steel body 4 having been seated within the mold 2 liquid or solid 45 copper 5 is filled in the spaces between. Heat is now applied from 7 until union is effected between the copper and steel.

What I claim is:

1. The process of making copper clad 50 steel which comprises contacting a body of steel with a body of copper on one side and applying heat to the other side of the steel body in amount sufficient to maintain the proximate layer of copper molten until a 55 union is effected the application of heat being in such manner as to maintain such proximate layer of copper at a higher temperature than the rest of the copper.

2. The process of making copper clad 60 steel which comprises contacting a tubular body of steel with a body of copper on one side and applying heat to the other side of the steel body in amount sufficient to maintain the proximate layer of copper

molten until a union is effected the application of heat being in such manner as to maintain such proximate layer of copper at a higher temperature than the rest of the copper.

3. The process of making copper clad 70 steel which comprises oxidizing one side of a body of steel, contacting the oxidized side with a body of copper and applying heat to the other side of the steel body till a union is effected.

4. The process of making copper clad 75 steel which comprises oxidizing one side of a tubular body of steel, contacting the oxidized side with a body of copper and applying heat to the other side of the steel body 80 till a union is effected.

5. The process of making copper clad 85 steel which comprises oxidizing one side of a body of steel by heating in an atmosphere of steam, contacting the oxidized side with a body of copper and applying heat to the other side of the steel body till a union is effected.

6. The process of making copper clad 90 steel which comprises oxidizing one side of a tubular body of steel by heating in an atmosphere of steam, contacting the oxidized side with a body of copper and applying heat to the other side of the steel body till a union is effected.

7. The process of making copper clad 95 steel which comprises contacting a body of steel with a solid body of copper on one side, and heating the other side of the steel body till the copper is melted and a union effected.

8. The process of making copper clad 100 steel which comprises contacting a tubular body of steel with a body of copper on one side, applying heat to the other side of the steel body in such amount and manner as to maintain the proximate layer of copper at a higher temperature than the rest of the copper and maintaining such application of heat until a weld union is effected between 105 the copper and the steel.

9. The process of making copper clad 110 steel which comprises oxidizing one side of a body of steel, contacting the oxidized side with a body of copper and applying heat 115 to the other side of the steel body till the copper is melted and a union effected.

10. The process of making copper clad 120 steel which comprises oxidizing one side of a tubular body of steel, contacting the oxidized side with a body of copper and applying heat to the other side of the steel body till the copper is melted and a union effected.

11. The process of making copper clad 125 steel which comprises oxidizing one side of a body of steel by heating in an atmosphere of steam, contacting the oxidized side with

a body of copper and applying heat to the other side of the steel body till the copper is melted and a union effected.

12. The process of making copper clad steel which comprises oxidizing one side of a tubular body of steel by heating in an atmosphere of steam, contacting the oxidized side with a body of copper and applying

heat to the other side of the steel body till the copper is melted and a union effected. 10

In testimony whereof, I affix my signature in the presence of witnesses.

WILLIAM MARSHALL PAGE.

Witnesses:

P. M. WEIS,

JOHN B. PATTON.